

Patented June 16, 1953

2,642,361

# UNITED STATES PATENT OFFICE

2,642,361

## PHOTOGRAPHIC SILVER HALIDE EMULSIONS SENSITIZED WITH WATER-IN-SOLUBLE GOLD COMPOUNDS

Rudolph E. Damschroder and Henry C. Yutzy,  
Rochester, N. Y., assignors to Eastman Kodak  
Company, Rochester, N. Y., a corporation of  
New Jersey

No Drawing. Application July 20, 1949,  
Serial No. 105,892

22 Claims. (Cl. 95—7)

1

This invention relates to the sensitization of photographic silver halide emulsions with water-insoluble gold compounds.

The usual procedure for preparing photographic silver halide developing-out emulsions, especially photographic gelatino-silver-halide developing-out emulsions comprises the following steps:

- (1) Precipitation, wherein the silver halide is precipitated by the interaction of a water-soluble silver salt and a water-soluble halide, in the presence of a carrier, e. g. gelatin.
- (2) Digestion, wherein the above precipitate is heated for a period of time at a raised temperature, e. g. 50° to 60° C., with or without the addition of further carrier, e. g. gelatin.
- (3) Washing, wherein the digested, solidified (e. g. by chilling) emulsion is washed to remove soluble salts.
- (4) Melting out and second digestion, wherein the washed emulsion is melted and the resulting flowable emulsion is heated for a period of time, with or without the addition of further carrier, e. g. gelatin.

Of course, variations of the above four steps can be employed. An emulsion, when used without employing a step, such as (3), we call an unwashed, finished emulsion. An emulsion, when used following completion of all four steps, we call a washed, finished emulsion. The latter is the type of emulsion generally used.

During the last step, i. e. the melting-out and second digestion, the emulsion increases in sensitivity. To increase the speed of photographic emulsions various substances have been added at various stages in the preparation of the emulsions. Usually the additions are made during one of the digestion periods. Frequently sulfur compounds, i. e. so-called "sulfur sensitizers" have been added, e. g. allyl isothiocyanate, thiourea, thiocarbanilide, etc., have been added. More recently, it has been proposed to employ ammonium and/or metal thiocyanates for this purpose. Still more recently water-soluble gold salts have been proposed for the same purpose.

We have now found that the sensitivity of photographic silver halide emulsions can be greatly increased by digesting the emulsions in the presence of water-insoluble gold compounds rather than water-soluble gold salts, even though the solubility of the gold compounds is so low that the concentration of gold ions in the emulsion (as compared with the concentration obtained when water-soluble gold salts are employed) is very low, indeed.

2

It is, accordingly, an object of our invention to provide an improved process for sensitizing photographic silver halide emulsions. Other objects will become apparent hereinafter.

In accordance with our invention, we incorporate in a photographic silver halide emulsion, before or during the final digestion, a water-insoluble gold compound which has a solubility in water not greater than the equivalent of 1.0 mg. of gold (metallic) per 100 ml. of water at 25° C. and digest the emulsion in the presence of the gold compound. Gold compounds having a solubility in water as low as the equivalent of 0.03 mg. per 100 ml. of water at 25° C. can be employed, as can gold compounds of still lower solubility.

Typical of such water-insoluble gold compounds are:

20 I



25 II



30 III



35 IV



V

50



55

3



Any other water-insoluble gold compound which has a solubility in water not greater than the equivalent of 1.0 mg. of gold per 100 ml. of water at 25° C. can be used in practicing our invention.

The water-insoluble gold compounds can be added to the emulsions, before or during the final digestion, in solution in suitable organic solvents or as colloidal dispersions. Typical organic solvents include acetic acid, acetone, pyridine, methyl alcohol, etc. Colloidal dispersions in gelatin, polyvinyl alcohol, partially hydrolyzed cellulose acetate, casein can be used.

Advantageously the level of pH during the digestion of the emulsion, in the presence of the gold compound, is maintained at or below 9, although this is not essential. Generally speaking the best results are obtained by digesting the emulsions at a pH of from 5 to 9, in the presence of the water-insoluble gold compound. Digestion of the emulsions in the presence of the gold compounds is advantageously effected at from 40° C. to 65° C., although other temperatures can be used. A temperature range of 50° to 60° C. ordinarily gives the best results.

Ordinarily, it is advantageous to employ a concentration of the water-insoluble gold compound equivalent to from 2.5 to 1000 mg. of gold per kilogram of silver nitrate used in preparing the emulsion; most advantageously a concentration of water-insoluble gold compound equivalent to from 2 to 30 mg. of gold per kilogram of silver nitrate used in preparing the emulsion is employed.

Advantageously, the emulsions are digested in the additional presence of at least one sulfur compound, e. g. a sulfur sensitizer, for instance an organic compound containing a C=S group

4

or a —C—S—S—C— group. Typical of such sulfur sensitizers are:



Normal gelatins contain small amounts of sulfur compounds, such as thiosinamine or allylisothiocyanate, but it is nevertheless frequently advantageous to add to the gelatin emulsions additional sulfur sensitizers. Beneficial effects are also obtained by adding to the emulsions at least one metal or ammonium thiocyanate, e. g. alkali metal thiocyanates (e. g. sodium or potassium thiocyanate) alkaline earth metal thiocyanates (e. g. calcium thiocyanate, strontium thiocyanate, etc.), cadmium thiocyanate, ammonium thiocyanate, etc. Of course, thiocyanates containing cations which cations are known to have, in themselves, a deleterious effect on silver halide emulsions should be avoided. Otherwise, the beneficial effects attained with the thiocyanate 35 would be partially nullified by the deleterious action of the cation. Thus, iron thiocyanate which contains the iron cation should be avoided. One or more sulfur sensitizers or one or more thiocyanates selected from the group consisting 40 of metal and ammonium thiocyanates can be employed. One or more sulfur sensitizers can be employed in conjunction with one or more thiocyanates containing a cation selected from the group consisting of metal and ammonium 45 cations. The sulfur sensitizers and thiocyanates are advantageously incorporated in the emulsions in the form of their solutions in a suitable solvent, such as water, methyl or ethyl alcohol.

The sulfur sensitizers can be incorporated in the emulsions at any stage of the preparation of the emulsions, e. g. during precipitation of the silver halides, during the first digestions (ripening) or during the second digestion of the emulsions. When incorporating metal and ammonium thiocyanates in the emulsions prior to washing, the amount can vary widely. Advantageously, however, an amount of thiocyanate equal to from about 10 to about 75 g. per kilogram of silver nitrate used in preparing the emulsion 60 is employed. If the thiocyanate or sulfur sensitizer is not added until later in the preparation, e. g. after washing, it is advantageous to employ, in the case of the thiocyanates, an amount equal to from about 0.1 to about 10 g. per kilogram of silver nitrate used in preparing the emulsion.

It is advantageous to digest, i. e. to heat treat the emulsion with both the water-insoluble gold compound and the sulfur sensitizer or thiocyanate present, at an appropriate temperature, e. g. at from 100 to 150° F. During digestion, i. e. the second digestion as contrasted with the first di-

gestion or ripening, the pH of the emulsion is advantageously adjusted to between 5 and 7. Maintenance of the emulsion on the acid side of neutrality during coating is also advantageous.

The following examples will serve to illustrate further the manner of practicing our invention.

**EXAMPLE 1**

A batch of gelatino-silver-bromoiodide emulsion was prepared as described by Trivelli and Smith, Phot. J. 79, 330 (1939), using a precipitation time of about 20 minutes (emulsion No. 11, page 330), except that just before the final digestion of the emulsion, sodium thiocyanate (1 g. per 1000 g. of silver nitrate used) was added to the emulsion. A portion of the emulsion so prepared was coated on cellulose acetate film and dried. The film was exposed in a 1b sensitometer at  $\frac{1}{25}$  second exposure, using 100 watt, sunlight quality illumination. The exposed film was then developed in Eastman Kodak Company's "D-19" developer for 4 minutes at 20° C. Results are recorded in the table below.

Further batches of gelatino-silver-bromoiodide emulsion were prepared as described by Trivelli and Smith, *supra*, using a precipitation time of about 20 minutes, except that in each case just before the final digestion of the emulsion, a water-insoluble gold compound which has a solubility in water not greater than the equivalent of 1.0 mg. of gold per 100 ml. of water at 25° C. was added to the emulsion together with sodium thiocyanate (1 g. per 1000 g. of silver nitrate used). A portion of each emulsion so prepared was coated on cellulose acetate film and dried. The dried films were exposed in a 1b sensitometer at  $\frac{1}{25}$  second exposure, using 100 watt, sunlight quality illumination. The exposed films were then developed in Eastman Kodak Company's "D-19" developer for 4 minutes at 20° C. Results are recorded in the following table.

Table

| Exposure time | g. of gold/1,000 g. AgNO <sub>3</sub> used in preparing emulsion | Speed (1/100 sec.) | Gamma | Fog  | Emulsion No. | Speed (1/100 sec.) | Gamma | Fog |
|---------------|------------------------------------------------------------------|--------------------|-------|------|--------------|--------------------|-------|-----|
| none          | none                                                             | 65                 | 1.06  | 0.04 |              |                    |       |     |
| II            | 0.006                                                            | 102                | 1.16  | 0.06 |              |                    |       |     |
| III           | 0.012                                                            | 90                 | 1.16  | 0.10 |              |                    |       |     |
| IV            | 0.006                                                            | 100                | 1.05  | 0.08 |              |                    |       |     |
| V             | 0.012                                                            | 82                 | 0.79  | 0.06 |              |                    |       |     |
| VI            | 0.006                                                            | 140                | 1.24  | 0.12 |              |                    |       |     |
| VII           | 0.012                                                            | 120                | 1.24  | 0.10 |              |                    |       |     |
| VIII          | 0.005                                                            | 100                | 1.10  | 0.07 |              |                    |       |     |
| IX            | 0.10                                                             | 92                 | 1.22  | 0.13 |              |                    |       |     |
| X             | 0.004                                                            | 102                | 0.89  | 0.04 |              |                    |       |     |
| XI            | 0.008                                                            | 88                 | 1.40  | 0.09 |              |                    |       |     |
| XII           | 0.0045                                                           | 92                 | 1.30  | 0.11 |              |                    |       |     |
| XIII          | 0.009                                                            | 84                 | 1.32  | 0.10 |              |                    |       |     |
| XIV           | 0.014                                                            | 108                | 1.21  | 0.04 |              |                    |       |     |

From the foregoing examples the marked increases in photographic speed that can be obtained in accordance with our invention are apparent.

Water-insoluble gold compounds which are advantageously employed in practicing our invention can be prepared as illustrated in the following examples.

**EXAMPLE 2**

A solution containing 1.61 g. of 3-ethyl-2-(3-ethyl-2-thiobenzothiazolylidene) rhodanine in 25 cc. of acetic acid was added to a hot suspension of 1.0 g. of auric chloride in 50 cc. of 95% ethyl alcohol. The reaction mixture was then cooled and the precipitated solid was collected, washed with 95% ethyl alcohol, and dried. The product was 3-ethyl-2-(3-ethyl-2-thiobenzothiazolylidene) auric chloride (CH<sub>3</sub>CH<sub>2</sub>CH<sub>2</sub>CSAuCl<sub>2</sub>), m.p. 180° C. (decompose-

5 A solution containing 1 g. of auric chloride in 5 cc. of 95% ethyl alcohol was added to 50 cc. of 95% ethyl alcohol containing 1.81 g. of 3-methyl-2-(3-thiobenzothiazolylidene) (prepared by heating 2-methylmercaptobenzothiazole metho-p-toluenesulfonate in boiling pyridine). The above formulated product separated as a white solid at once. The reaction mixture was stood at about 20° C. for several hours and then chilled. The white solid was filtered from the chilled mixture and washed on the filter with 95% ethyl alcohol. The yield of colorless crystals was 98% crude, and 73% after one recrystallization from acetic acid.

**EXAMPLE 3**

15 A solution containing 1.61 g. of 3-ethyl-2-(3-ethyl-2-thiobenzothiazolylidene) rhodanine in 25 cc. of acetic acid was added to a hot suspension of 1.0 g. of auric chloride in 50 cc. of 95% ethyl alcohol. The reaction mixture was then cooled and the precipitated solid was collected, washed with 95% ethyl alcohol, and dried. The yield of colorless crystals was 98% crude, and 73% after one recrystallization from acetic acid.

20

25

30

35

40

45

50

55

60

65

70

75



A solution containing 0.33 g. of auric chloride in 10 cc. of 95% ethyl alcohol was added to 100 cc. of 95% ethyl alcohol containing 0.85 g. of 3-ethyl-2-(3-thiobenzothiazolylidene) rhodanine (prepared by heating 3-ethylrhodanine and o-aminobenzaldehyde in acetic acid solution according to Gränacher et al., *Helv. Chim. Acta* 8, 890 (1925)). The above-formulated compound precipitated and after the reaction mixture stood for several hours at 20° C., the product was collected on a filter and washed with 95% ethyl alcohol. The yield of light cream crystals was 75% after one recrystallization from acetic acid.

**EXAMPLE 4**

45 A solution containing 0.34 g. of auric chloride in 10 cc. of 95% ethyl alcohol was added to a solution containing 1.11 g. of 3-ethyl-5-[3-ethyl-2-(3-ethyl-2-thiobenzothiazolylidene) ethylidene]rhodanine in 25 cc. of pyridine and 25 cc. of 95% ethyl alcohol. A reddish solid separated at once. The reaction mixture was stood at about 20° C. for several hours and then the solid was collected on a filter and washed with 95% ethyl alcohol. The yield of product was 63% crude and 12% after two recrystallizations from nitromethane. The reddish crystals had melting point 231-232° C. with decomposition.



50 A solution containing 0.5 g. of auric chloride in 10 cc. of 95% ethyl alcohol was added to a hot suspension of 1.61 g. of 3-ethyl-5-[3-ethyl-2-(3-ethyl-2-thiobenzothiazolylidene) ethylidene]rhodanine in 25 cc. of acetic acid. The reaction mixture was stood several hours at about 20° C. and the precipitated solid was filtered off and washed on the filter with 95% ethyl alcohol. The washed solid was extracted with 180 cc. of hot nitromethane. Upon chilling the hot extract, the crystals which formed were

**EXAMPLE 5**

55 A solution containing 0.5 g. of auric chloride in 10 cc. of 95% ethyl alcohol was added to a hot suspension of 1.61 g. of 3-ethyl-5-[3-ethyl-2-(3-ethyl-2-thiobenzothiazolylidene) ethylidene]rhodanine in 25 cc. of acetic acid. The reaction mixture was stood several hours at about 20° C. and the precipitated solid was filtered off and washed on the filter with 95% ethyl alcohol. The washed solid was extracted with 180 cc. of hot nitromethane. Upon chilling the hot extract, the crystals which formed were



filtered off and recrystallized from 155 cc. of nitromethane. The yield of golden-yellow crystals was almost 100%.

## EXAMPLE 6



suspension of 1.18 g. of 3,3'-diethyl-4,5,4',5'-di-benzothiacyanine chloride in 40 cc. of absolute ethyl alcohol. A dark solid was formed at once. After chilling for one hour at 0° C. the solid was collected on a filter and washed with absolute ethyl alcohol. The yield was 93% crude and 74% after one recrystallization from nitromethane. The blue crystals gave a yellow solution in acetone.

## EXAMPLE 10



A solution containing 1 g. of auric chloride in 10 cc. of absolute ethyl alcohol was added to a suspension of 0.92 g. of 1,3-diethylthia-2'-cyanine chloride in 20 cc. of absolute ethyl alcohol. An orange solid separated at once. After chilling for one hour at 0° C., the solid was collected on a filter and washed with absolute ethyl alcohol. The yield of dye was 89% crude and 71% after one recrystallization from nitromethane. The reddish coppery needles gave an amber solution in acetone.

## EXAMPLE 11



A solution containing 1 g. of auric chloride in 10 cc. of absolute ethyl alcohol was added to a suspension of 0.93 g. of 3,3'-diethylthiacyanine chloride in 20 cc. of absolute ethyl alcohol. A pale orange solid separated at once. After chilling for one hour at 0° C., the solid was collected on a filter and washed with absolute ethyl alcohol. The yield of dye was 56% crude and 38% after one recrystallization from nitromethane. The deep red crystals with a blue reflex gave a pale yellow solution in acetone.

In a manner similar to that shown in Examples 2 to 11, other similar organic water-insoluble gold compounds can be prepared. In the benzene nuclei of the organic gold compounds set forth in Examples 2 to 11, one or more of the hydrogen atoms can be replaced by a chlorine, a bromine or an iodine atom or by an alkyl or aryl group, e. g. methyl, ethyl, phenyl, etc. The preparation of  $\text{Au}_2\text{S}$  is described for example by J. W. Mellor, "A Comprehensive Treatise on Inorganic Chemistry," vol. III, page 611; by E. A. Schneider, Ber. 24, 2241 (1891) and by Gmelin-Kraut, V2, page 267A(a). The preparation of  $\text{Au}_2\text{Se}$  is described by Abegg and Overbach, "Handbuch der Anorg. Chem., vol. II, part 1, page 822, and by Gmelin-Kraut, V2, page 271(A). The preparation of  $\text{AuI}$  is described by Mellor, loc. cit., page 608, and by Gmelin-Kraut, V2, page 282.

Sensitizing dyes of all types can be employed to spectrally (optically) sensitize our new emulsions, e. g. erythrosin, Congo red, any of the sensitizing cyanine dyes (monomethine, trimethine, pentamethine, heptamethine, etc.), any of the sensitizing merocyanine dyes (see United States Patent 2,078,233, dated April 27, 1937, for example), any of the sensitizing hemicyanine

## EXAMPLE 9



A solution containing 1 g. of auric chloride in 10 cc. of absolute ethyl alcohol was added to a

dyes (see United States Patent 2,166,736, dated July 18, 1939, for example), any of the sensitizing hemioxonol dyes (see United States Patent 2,216,441, dated October 1, 1940, and United States Patent 2,165,339, dated July 11, 1939, for example), etc.

Photographic elements comprising our new emulsions can be made up in the usual manner by coating the flowable emulsions on to a support of a suitable material, such as glass, photographic paper, cellulose derivative or resin film, etc. to desired thickness, and then setting and drying the coated emulsion.

Our new emulsions can contain hardening agents, setting agents, stabilizing agents, super-sensitizing combinations of sensitizing dyes or a supersensitizing combination of one or more sensitizing dyes and another substance.

Eastman Kodak Company's "D-19" developer has the following composition:

|                                |        |       |
|--------------------------------|--------|-------|
| Water                          | liters | 2.0   |
| N-methyl-p-aminophenol sulfate | grams  | 8.8   |
| Sodium sulfite, desiccated     | do     | 384.0 |
| Hydroquinone                   | do     | 35.2  |
| Sodium carbonate, desiccated   | do     | 192.0 |
| Potassium bromide              | do     | 20.0  |
| Water to make                  | liters | 4.0   |

Materials other than gelatin can be employed as the carrier for the silver halide in practicing our invention. Among the non-gelatin silver halide emulsions are silver halide emulsions prepared using as the vehicle or carrier polyvinyl alcohol ("polyvinyl alcohol" is herein intended to include all water-soluble hydrolyzed polyvinyl esters containing an ester group content equivalent to from 0 to 5% by weight of polyvinyl ester); silver halide emulsions prepared using as the vehicle or carrier hydrolyzed polyvinyl acetate containing an acetate group content equivalent to from 59 to 71% by weight of polyvinyl acetate; silver halide emulsions prepared using as the vehicle or carrier polyvinyl acetals containing a large proportion of polyvinyl alcohol hydroxyl groups, e. g. polyvinyl acetaldehyde acetals containing polyvinyl acetaldehyde acetal groups equivalent to at least 50% by weight of polyvinyl acetaldehyde acetal and polyvinyl alcohol hydroxyl groups equivalent to at least 15% by weight of polyvinyl alcohol, polyvinyl propionaldehyde acetals containing polyvinyl alcohol hydroxyl groups equivalent to from 45 to 60% by weight of polyvinyl alcohol, and polyvinyl butyraldehyde acetals containing polyvinyl alcohol hydroxyl groups equivalent to from 60 to 80% by weight of polyvinyl alcohol, etc. Any polyvinyl compound, especially those containing only carbon, hydrogen and oxygen atoms, or those containing carbon, hydrogen, oxygen and amine nitrogen atoms or ammonium nitrogen atoms, which is soluble in a mixture of ethyl alcohol and water (containing from 0 to 50% by volume of ethyl alcohol) to the extent of 10 g. per 100 g. of solvent can be employed as the vehicle or carrier in preparing our non-gelatin silver halide emulsions. Moreover, any other resinous or colloidal material soluble in an ethyl alcohol-water mixture or in water, as stated above, can be employed in preparing our non-gelatin silver halide emulsions, e. g. soluble polyamide resins, such as described in United States Patent 2,384,072, dated September 4, 1945, and hydrolyzed copolymers of vinyl esters and ethylene or propylene, such as described in United States Patent 2,397,866, dated April 2, 1946. Still fur-

ther examples of colloidal materials which can be employed as vehicles or carriers in preparing our non-gelatin emulsions are hydrolyzed cellulose carboxylic esters, such as hydrolyzed cellulose acetate or hydrolyzed cellulose acetate propionate, containing from 19 to 33% by weight of acyl groups, for example. Any cellulose compound, especially those containing only carbon, hydrogen and oxygen atoms, or those containing only carbon, hydrogen, oxygen and amino nitrogen atoms or ammonium nitrogen atoms, which is soluble in a mixture of ethyl alcohol and water (containing from 0 to 50% by volume of ethyl alcohol) to the extent of 10 g. per 100 g. of solvent can be employed as the vehicle or carrier in preparing our non-gelatin silver halide emulsions.

In connection with the non-gelatin colloidal materials, such as polyvinyl alcohol, the silver halide emulsions can be prepared using gelling agents, such as phenols, e. g. orcinol, gallic acid, 2,4-dihydroxybenzoic acid, 4-chlororesorcinol,  $\alpha$ -naphthol, phloroglucinol, 2,7-dihydroxynaphthalene, etc. Moreover, the non-gelatin silver halide emulsions can be prepared using silver halide dispersing agents, e. g. starch acetate, gum arabic, a copolymer of maleic anhydride and vinyl acetate, low viscosity methyl cellulose, water-soluble amino carbohydrate dispersing agents (e. g. diethanolamine cellulose acetate or any other of these agents described in United States Patent 2,360,238, dated October 10, 1944) amino resin dispersing agents (e. g. dimethylaminobenzaldehyde acetals of polyvinyl alcohol, or water-soluble polyvinyl acetals in which at least a part of the acetal groups are 4-formylphenyltrialkylammonium salt acetal groups, such as the polyvinyl acetal of 4-formylphenyl trimethylammonium methylsulfate and other such compounds described in United States Patent 2,358,836, dated September 26, 1944), etc.

Polyvinyl compound silver halide emulsions and their preparation are described in United States Patents 2,286,216, dated June 16, 1942; 2,276,322, dated March 17, 1942; 2,276,323, dated March 17, 1942; 2,311,058, dated February 16, 1943; 2,311,059, dated February 16, 1943; 2,367,511, dated January 16, 1945; 2,376,371, dated May 22, 1945 and 2,110,491, dated March 8, 1938.

Non-gelatin proteins can also be employed as vehicles or carriers in preparing the silver halide emulsions which are sensitized in accordance with our invention. Proteins, such as casein, soybean protein, blood albumin, egg albumin, castor bean protein, globulin and edestin are examples of such non-gelatin proteins. Non-gelatin proteins which have been converted to a derivative thereof, e. g. by reaction with a sulfonyl chloride, a carboxylic chloride, a carboxylic anhydride, an isocyanate, a 1,4-diketone or acrylonitrile, and then oxidized, e. g. with hydrogen peroxide, as described in the copending application of Wesley G. Lowe and John W. Gates, Jr. Serial No. 768,480, filed August 13, 1947, can also be employed.

Our invention is directed especially to the sensitization of photographic silver halide emulsions in which the silver halide is principally silver bromide, but can be employed with any silver halide emulsion, particularly the customary silver chloride, silver chlorobromide, silver chlorobromoiodide, silver chloroiodide, silver bromide and silver bromoiodide developing-out emulsions. By the term "photographic silver halide emulsion in which the silver halide is prin-

incipitally silver bromide," we mean a photographic silver halide emulsion in which from 60 to 100% of the weight of the silver halide is silver bromide.

What we claim as our invention and desire to be secured by Letters Patent of the United States is:

1. A process for sensitizing a photographic silver halide emulsion comprising adding to the emulsion, before or during final digestion, a water-insoluble gold compound which has a solubility in water equivalent to from 0.03 mg. to 1.0 mg. of gold per 100 ml. of water at 25° C., and digesting the emulsion in the presence of the water-insoluble gold compound.

2. A process for sensitizing a photographic silver halide developing-out emulsion comprising adding to the emulsion, before or during final digestion, a water-insoluble gold compound which has a solubility in water equivalent to from 0.03 mg. to 1.0 mg. of gold per 100 ml. of water at 25° C., and digesting the emulsion in the presence of the water-insoluble gold compound.

3. A process for sensitizing a photographic gelatino-silver-halide developing-out emulsion comprising adding to the emulsion, before or during final digestion, a water-insoluble gold compound which has a solubility in water equivalent to from 0.03 mg. to 1.0 mg. of gold per 100 ml. of water at 25° C., and digesting the emulsion in the presence of the water-insoluble gold compound.

4. A process for sensitizing a photographic gelatino-silver-halide developing-out emulsion in which the silver halide is principally silver bromide comprising adding to the emulsion, before or during final digestion, a water-insoluble gold compound which has a solubility in water equivalent to from 0.03 mg. to 1.0 mg. of gold per 100 ml. of water at 25° C., and digesting the emulsion in the presence of the water-insoluble gold compound.

5. A process for sensitizing a photographic gelatino-silver-halide developing-out emulsion in which the silver halide is principally silver bromide comprising adding to the emulsion, before or during final digestion, a sulfur sensitizer and a water-insoluble gold compound which has a solubility in water equivalent to from 0.03 mg. to 1.0 mg. of gold per 100 ml. of water at 25° C., and digesting the emulsion in the presence of the gold compound and the sulfur sensitizer.

6. A process for sensitizing a photographic gelatino-silver-halide developing-out emulsion in which the silver halide is principally silver bromide comprising adding to the emulsion, before or during final digestion, a sulfur sensitizer and a water-insoluble gold compound which has a solubility in water equivalent to from 0.03 mg. to 1.0 mg. of gold per 100 ml. of water at 25° C., and digesting the emulsion in the presence of the gold compound and the sulfur sensitizer, on the acid side of neutrality.

7. A process for sensitizing a photographic gelatino-silver-halide developing-out emulsion in which the silver halide is principally silver bromide comprising adding to the emulsion, before or during final digestion, an alkali metal thiocyanate and a water-insoluble gold compound which has a solubility in water equivalent to from 0.03 mg. to 1.0 mg. of gold per 100 ml. of water at 25° C., and digesting the emulsion in the presence of the gold compound and the thiocyanate, on the acid side of neutrality.

8. A process for sensitizing a photographic gelatino-silver-halide developing-out emulsion in which the silver halide is principally silver bromide comprising adding to the emulsion, before or during final digestion, sodium thiocyanate and a water-insoluble gold compound which has a solubility in water equivalent to from 0.03 mg. to 1.0 mg. of gold per 100 ml. of water at 25° C. and digesting the emulsion in the presence of the gold compound and the thiocyanate, on the acid side of neutrality.

9. A process for sensitizing a photographic gelatino-silver-halide developing-out emulsion in which the silver halide is principally silver bromide comprising adding to the emulsion, before or during final digestion, sodium thiocyanate in a concentration of from 0.1 to 10 grams per kilogram of silver nitrate employed in preparing the emulsion and a water-insoluble gold compound which has a solubility in water equivalent to from 0.03 mg. to 1.0 mg. of gold per 100 ml. of water at 25° C., in a concentration of from 2.5 to 30 mg. per kilogram of silver nitrate employed in preparing the emulsion, and digesting the emulsion in the presence of the thiocyanate and the gold compound on the acid side of neutrality.

10. A process for sensitizing a photographic gelatino-silver-bromoiodide developing-out emulsion comprising adding to the emulsion, before or during final digestion, sodium thiocyanate in a concentration of from 0.1 to 10 grams per kilogram of silver nitrate employed in preparing the emulsion and aurous sulfide (Au<sub>2</sub>S) in a concentration of from 2.5 to 30 mg. per kilogram of silver nitrate employed in preparing the emulsion, and digesting the emulsion in the presence of the thiocyanate and the aurous sulfide on the acid side of neutrality.

11. A process for sensitizing a photographic gelatino-silver-bromoiodide developing-out emulsion comprising adding to the emulsion, before or during final digestion, sodium thiocyanate in a concentration of from 0.1 to 10 grams per kilogram of silver nitrate employed in preparing the emulsion and the gold compound represented by the following formula:



in a concentration of from 2.5 to 30 mg. per kilogram of emulsion employed in preparing the emulsion, and digesting the emulsion in the presence of the thiocyanate and the gold compound on the acid side of neutrality.

12. A process for sensitizing a photographic gelatino-silver-bromoiodide developing-out emulsion comprising adding to the emulsion, before or during final digestion, sodium thiocyanate in a concentration of from 0.1 to 10 grams per kilogram of silver nitrate employed in preparing the emulsion and the gold compound represented by the following formula:



in a concentration of from 2.5 to 30 mg. per kilogram of silver nitrate employed in preparing the emulsion, and digesting the emulsion in the presence of the thiocyanate and the gold compound on the acid side of neutrality.

13. A process for sensitizing a photographic gelatino-silver-bromoiode developing-out emulsion comprising adding to the emulsion, before or during final digestion, sodium thiocyanate in a concentration of from 0.1 to 10 grams per kilogram of silver nitrate employed in preparing the emulsion and the gold compound represented by the following formula:



in a concentration of from 2.5 to 30 mg. per kilogram of silver nitrate employed in preparing the emulsion, and digesting the emulsion in the presence of the thiocyanate and the gold compound on the acid side of neutrality.

14. A process for sensitizing a photographic gelatino-silver-bromoiode developing-out emulsion comprising adding to the emulsion, before or during final digestion, sodium thiocyanate in a concentration of from 0.1 to 10 grams per kilogram of silver nitrate employed in preparing the emulsion and the gold compound represented by the following formula:



in a concentration of from 2.5 to 30 mg. per kilogram of silver nitrate employed in preparing the emulsion, and digesting the emulsion in the presence of the thiocyanate and the gold compound on the acid side of neutrality.

15. A process for sensitizing a photographic silver halide emulsion comprising digesting the emulsion in the presence of a water-insoluble gold compound which has a solubility 10 in water equivalent to from 0.03 mg. to 1.0 mg. of gold per 100 ml. of water at 25° C.

16. The photographic emulsion obtained according to the process of claim 1.

17. The photographic emulsion obtained according to the process of claim 15.

18. The photographic emulsion obtained according to the process of claim 10.

19. The photographic emulsion obtained according to the process of claim 11.

20 20. The photographic emulsion obtained according to the process of claim 18.

21. The photographic emulsion obtained according to the process of claim 12.

22. The photographic emulsion obtained according to the process of claim 14.

RUDOLPH E. DAMSCHRODER.  
HENRY C. YUTZY.

**References Cited in the file of this patent**

UNITED STATES PATENTS

Number Name Date  
2,399,083 Waller et al. Apr. 23, 1946

## FOREIGN PATENTS

35 Number Country Date  
608,667 Great Britain ----- Sept. 20, 1948

#### OTHER REFERENCES

40 Bureau of Standards Journal of Research, vol. 1, October 1928, pages 565-588; pages 575-588 particularly cited.